

Patented Jan. 22, 1929.

## UNITED STATES PATENT OFFICE.

HOWARD J. BLAKE, OF BOSTON, MASSACHUSETTS.

## MATRIX BOARD.

Application filed December 12, 1925. Serial No. 75,144.

No Drawing.

- The invention relates to improvement in matrix board for stereotypers use. The board as ordinarily used for stereotype purposes is usually composed of a mixture of fibre and a filler of some material, the mixture usually consisting of about 70% fibre and 30% of a clay filler. The board is usually made in sheet form called a mat or flong and sold to the stereotypers in this condition. This mat or sheet material is cut up as desired into blanks according to the size desired by the stereotyper. The impression for the matrix is then formed in the surface of the blank by suitable dies. After a few casts have been taken on the matrix, the surface becomes worn so that it is impossible to take any more good casts. The life of the matrix is usually sufficient to take only about six good casts.
- The object of the present invention is to provide a protective coating for the matrix board to give it greater wearing qualities so that there may be obtained a much greater number of casts. Preferably this coating is applied to the matrix board in its sheet form at the factory before it has been cut up into blanks for the stereotyper's use and before it has been subjected to the matrix forming dies.
- Another object of the invention is to provide this protective coating of such a character that it will readily take the impression of the dies to form the matrix and yet be sufficiently tough so that it will not crack or break under the forming pressure of the matrix dies and will have great wearing qualities in taking casts. The invention consists essentially in providing the matrix board with a homogeneous layer of cellulose xanthate.
- In producing the coated matrix board, I proceed as follows:
- Taking a sheet of plain matrix board as it comes from the mill; I then prepare the coating material as follows:
- I take commercially pure cellulose preferably wood pulp and first treat it with a solution of sodium hydroxide, preferably a 17.5% to 20% solution at ordinary room temperature of from 60° to 70° F. This treatment is preferably done by immersing the cellulose in sodium hydroxide or caustic soda and allowing it to soak in long enough to give a good mixture. This treatment is continued for some length of time, preferably about twenty-four hours, until it absorbs somewhat more than three times its own weight of the caustic soda, then the excess caustic is pressed out until the mixture weighs about four times the weight of the original cellulose before it was treated with the sodium hydroxide solution. For instance, if we start with ten pounds of pure cellulose, the resulting product, after being treated with the sodium hydroxide solution and after the excess caustic has been pressed out, should weigh about forty pounds.
- This resulting mixture is called soda cellulose and should be allowed to stand for several days for aging purposes, preferably some 90 to 100 hours, depending upon the variety of stock used. After it has been sufficiently aged, there is added to the mixture a quantity of carbon disulphide, preferably in weight about one-half of the weight of the original cellulose; for instance if we start with ten pounds of cellulose there should be now added about five pounds of carbon disulphide. This mixture should be agitated by stirring or by other means until the particles are all thoroughly mixed and gathered together, the time required for this being usually about five hours. Any suitable agitating machine or apparatus may be employed for this purpose.
- After the mixture has been suitably agitated there should be added sufficient water to make a substantially 6% viscous solution of the original cellulose. The percentage of solution may be varied according to judgment and may be more or less than 6%. It might properly be even as much as 10% or slightly more or even less than 6%. A considerable variation may be made and still obtain good results. This produces a cellulose xanthate solution commonly called viscose and which I use for the coating.
- The solution should then be diluted until it has the consistency of paint. The mixture is now ready to be applied to the surface of the matrix board. It may be applied in any suitable way to make a smooth, even coating like a coating of paint. It may be applied by the use of a brush or by any other suitable means, either by hand or by machine. After the coating has been applied, it should be allowed to dry in a temperature of about 68° F. After it is dry, the board is then ready for the stereotyper's use.
- The treatment of the matrix board with the above described coating preparation gives to the board a homogeneous layer of cellulose xanthate which will adhere firmly to the

board as firmly as though it were an integral part thereof. It forms a surface coating without impregnating the body of the matrix board.

5. The coating produced and applied as above described will harden when dry, being much harder than the surface of the uncoated board or mat and is ready for the stereotyper.

What I claim is:

10 1. A fibrous flong or mat for a matrix blank having a coating consisting of thio-carbonate

of cellulose otherwise known as cellulose xanthate.

2. A wood fibre flong or mat for a matrix blank having a surface coating of thio-carbonate of cellulose otherwise known as cellulose xanthate. 15

3. A paper board flong or mat for a matrix blank having a non-impregnating coating of thio-carbonate of cellulose. 20

In testimony whereof I affix my signature.

HOWARD J. BLAKE.